# EUROPEAN PATENT SPECIFICATION

(11) **EP 0 054 586 B1**
(45) Date of publication and mention of the grant of the patent: **08.05.1985**
(21) Application number: 80304611.9
(22) Date of filing: 19.12.1980
(51) Int. Cl.: B27N 3/14

(54) **Method and apparatus for orientation and deposition of fibres in the manufacture of fibreboard**
Verfahren und Vorrichtung zum Ausrichten und Ablagern der Fasern bei der Faserplattenherstellung
Procédé et dispositif pour orienter et déposer des fibres lors de la fabrication de plaques en fibre

(43) Date of publication of application: 30.06.1982
(73) Proprietor: MORRISON-KNUDSEN FOREST PRODUCTS COMPANY, INC., Boise Idaho 83729 (US)
(72) Inventor: Peters, Thomas E., Boise Idaho 83705 (US); Bleymaier, Joseph S. c/o Morrison Knudsen, Baltimore Maryland 21207 (US)
(74) Representative: Jones, Colin

## Description

This invention relates to fibreboard manufacture and, more particularly, to orientation and deposition of fibres in continuous-line formation of fibreboard having physical properties that are stronger in one direction.

Particleboards made from wood flakes, chips, and the like have been largely limited to floor underlay or furniture core uses. However, wood materials used for structural purposes take into consideration inherent directional properties of wood in its various levels of organization to provide adequate strength to handle long-term loads under a variety of conditions.

Sawn timber in its various structural uses takes advantage of the orthotropic nature of wood. However, sawn timber utilizes only a fraction of the forest resources; a significant portion remains as residual. Some of the residual may be converted to pulp and paper or comminuted wood panel product.

In the manufacture of panel product, wood particles have been assembled in a random fashion due to the nature of the processes used. However, the properties of a comminuted wood panel can be greatly affected by orientation of elongated wood particles in a preferred direction. As the degree of orientation increases, the panel properties exhibit more of the orthotropic properties of timber because of better alignment of the longest dimension of such wood particles with the grain direction.

Methods and apparatus have been advanced for use in alignment of certain wood particles. However, the particulate furnish produced from selected cellulosic raw materials by attrition in disc-refiners using heat or steam at atmospheric or elevated pressures is difficult to handle and orient properly. It is light in weight, about 16 to about 64 kg m-³ (one pound to four pounds per cubic foot), with the bulk of the furnish comprising extremely fine, hair-like fibres. It has not been practicable when working with such lightweight fibrous furnish to obtain desired levels of fibre orientation and uniformity at commercially economic production rates with prior art methods and apparatus.

Orientation chambers have been equipped with electrically charged walls, and/or partitions, arranged in vertically perpendicular relationship to a horizontal deposition surface, for electrostatic orientation purposes. However, charged fibres adhere to such planar electrodes and protrude such that build-up occurs. This build-up eventually reaches a point where the mass becomes too great and random avalanching onto the mat surface occurs. As a result, neither the appearance of, nor the weight distribution in, the mat is uniform.

In US-A-4113812 there is described a continuous-line method for orienting and depositing lightweight furnish, including fibrous material with curable binder, in the manufacture of fibreboard having directional properties, in which a web presenting an extended surface area for deposition of furnish is moved continuously in a forming direction, and lightweight furnish, including elongated fibres moving along a flow path which is substantially normal to said surface for deposition of furnish, is guided towards said web, and in which said fibres being so guided and deposited are oriented by utilizing electrical forces, tending to orient longitudinal axes of the elongated fibres in parallel relationship to the plane of the mat being formed and aligned with the forming direction, and said electrical forces are produced by virtue of electrical potentials established between a plurality of elongate roller electrodes disposed transversely to the forming direction and in spaced relationship from each other along the forming direction, the roller electrodes being disposed adjacent to the mat being formed.

US-A-4113812 does diclose the use of roller electrodes but these make electrical contact with the mat being formed and do not avoid the use of separate means, such as plate electrodes, for orienting the fibres as they descend along their flowpath.

An object of the present invention is to avoid the drawbacks and disadvantages of the prior art in providing desired orientation of fibres and uniformity of deposition at production rates which are commercially economic.

According to the present invention the roller electrodes are controllably rotated about their respective axes at a speed coordinated with the rate of longitudinal movement of the- web to deposit onto the mat being formed fibres which have been attracted to the roller electrodes and have adhered to the roller electrodes.

The invention also relates to apparatus for carrying out the above method in the continuous-line manufacture of fibreboard from lightweight furnish including fine textured elongated fibres and curable binding material, comprising a forming conveyor including a continuously moving web presenting an extended surface area for deposition of furnish, means for establishing a flow path and delivering the furnish for deposition with the fibres in discrete form substantially free of fibre clusters, a plurality of elongated electrically conductive roller electrodes located in the flow path of the furnish towards the surface area for deposition and in preselected spaced relationship above the surface area for deposition, the roller electrodes being mounted with their longitudinal axes in transverse relationship to the direction of movement of the surface area for deposition and in substantially parallel relationship to such surface area, whereby the roller electrodes are adjacent to a mat-forming surface presented by deposition of fibres on the surface area for deposition, and being spaced along-the direction of movement of such surface area across the flow path of furnish in approaching deposition, and means for applying an electrical potential to the roller electrodes for establishing an electric field having lines of force which tend to align longitudinal axes of the fibres with the direction of movement of the surface of deposition and into substantially parallel relationship with the mat-forming surface. The apparatus of the invention is characterised in that it includes means for controlling the electrical potential of the roller electrodes and means for rotating the roller electrodes at a speed coordinated with the speed of movement of the web such that elongated fibres adhering electrostatically to the roller electrodes contact the mat-forming surface upon rotation of the roller electrodes.

Thus, the roller electrodes utilized in the present invention are in the form of rods which are positively rotated.

Fibres, presented in individualized form, are attracted towards the rods and the mat being formed; orientation and deposition of the fibres are controlled by a combination of electrical and mechanical forces.

Thoses fibres which are electrically attracted to the rods adhere in spike-like fashion to the rods. Rotation of the rods and movement of the mat-forming surface are controlled so as to brush the fibres against the mat surface presented. Contact with the mat surface and centrifugal force created by rotation of the rods break the electrical adhesion to the rods and the fibres are deposited in a controlled manner to help attain a desired orientation ratio.

In addition, control of electrical polarity and the placement of the rods establish an electric field with lines of force extending in the machine- forming direction and substantially parallel to the forming surface on which the furnish is deposited. This electric field exerts a torque on the fibres approaching and falling between the rods tending to align axes of the fibres in the direction of movement of the mat forming surface and parallel to that surface.

The invention is further described by way of example with reference to the accompanying drawings, in which:
Figure 1 is a schematic view of apparatus for continuous-line manufacture of fibreboard in accordance with the present invention;
Figure 2 is a schematic view in cross-section, taken along the machine forming direction, of orientation and deposition means of the apparatus;
Figure 3 is a schematic representation in cross section along the machine forming direction of the electric field produced in the apparatus;
Figure 4 is a schematic representation in cross section along the machine forming direction of the effect of the electric field on the fibrous material; and
Figure 5 is a view in elevation showing structure for placement and rotation of the electrostatic field producing means of the apparatus.

In the handling of the lightweight furnish before fibre orientation, the furnish is metered, distributed and separated into discrete fibres as it approaches the orientation and deposition apparatus. In the continuous-line apparatus for manufacture of fibreboard shown in Fig. 1, a furnish supply 10 is located in vertically spaced relationship above a forming conveyor 11 presenting a web 12 on which a mat of the fibrous material is to be formed. From the furnish supply 10, the furnish descends into distribution means 14 for distribution transverse to the direction of movement of furnish towards web 12; e.g. distribution means 14 imposes a substantially uniform distribution of furnish over a distance correlated to the lateral dimension of the board measured in the plane of the board perpendicularly to the machine forming direction (indicated by arrow 26).

The laterally distributed furnish is accumulated in a feed chamber 16 and moved forward towards the web 12 by metering means 18. The metered furnish is distributed, in the direction of web travel, by longitudinal distribution means 20 over a preselected dimension which, with the established lateral dimension, determines the area of deposition of the mat-forming fibrous material.

The furnish, substantially uniformly distributed over the preselected area for deposition, moves in the direction of the web 12 through fibre separation means 22. Fibre clusters are broken up into discrete fibres by passage through the fibre separation means 22 as the furnish is delivered in the direction of web 12.

Furnish feed, distribution, metering, and fibre separation means are provided to deliver furnish at a suitable production flow rate over the area of deposition with the discrete fibres moving in the direction of the mat-forming surface substantially free of air turbulence effects.

The fibres move through an open-ended flow-through chamber 24 for orientation and deposition; the web 12 is moving in a continuous manner in the machine forming direction, as indicated by arrow 26, under the control of guide and drive roll means. The mat formed on the continuous web 12 then moves onto a conveyor 28 for transfer to a press; typically, the mat is subjected to heat and pressure which will polymerise a binder system; at the same time the mat is compressed into desired board density.

The furnish is moved through the orientation and deposition chamber 24 substantially free of pneumatic turbulence which would have an undesirable effect on orientation. The electrical forces imposed by energizing rod electrodes (to be described) in chamber 24 tend to orient the fibres in the plane of the fibreboard mat and with longitudinal axes of the fibres substantially aligned with the forming direction. A combination of electrical and mechanical forces is used to achieve desired orientation and substantially uniform deposition over the predetermined area.

Referring to Fig. 2, the orientation and deposition chamber 24 includes guide walls defining an open-ended flow-through structure into which the furnish is moving as indicated by arrow 30. The guide walls of the flow-through chamber define the area of deposition. Referring to the direction of movement of web 12 indicated by arrow 26, guide wall 32 is located at the leading end of the area of deposition and guide wall 34 is located at the trailing end of the area of deposition.

Desired orientation is carried out uniformly over the full area of deposition. Electrically conductive rods 36 to 41 are selectively positioned and supported in close proximity to the web 12. The rods 36 to 41 are elongated with their longitudinal axes disposed in transverse relationship to the forming direction and parallel to the deposition area. Electrical polarity of the rods is selected; in the preferred embodiment, the rods 36 to 42 are electrically charged so that, at any instant, each next adjacent rod is of opposite polarity; for example, rod 36 is connected to be of positive polarity while rod 37 is connected to be of negative polarity.

The electrically charged elongated rods 36 to 41 are predeterminedly spaced above web 12 in the direction of approach of furnish. Each rod is contiguous to the mat-forming surface on web 12 with the predetermined spacing of the rods from the surface of web 12 taking into account the increasing thickness of the mat as the web 12 travels longitudinally towards the leading end of the structure 24. Therefore, rods located near the leading end of the area of deposition in structure 24 will be spaced a greater distance above the support surface of the web 12 of the transport conveyor than those at the trailing end of the area of deposition. The contiguous relationship of the peripheral surface of the rods and the exposed surface of the mat being formed remains substantially the same regardless of the depth of the mat.

The web 12 of the forming conveyor can comprise a continuous foraminous belt woven from nylon or similar material. Support and electrical contact of the undersurface of web 12 is achieved with electrical conductor bars 44 to 49 which are elongated with their longitudinal axes extending in transverse relationship to the direction of movement of the web 12. Preferably these bars present a flat surface for support of the web. In the array shown, such bars are connected so that each next adjacent bar, at any instant, is of opposite polarity; for example, bar 44 is positive and bar 45 is negative, etc.

Although web 12 is essentially non-conductive, the voltage level is such that a small current is established through the fibre mat and the forming belt. Dielectric properties of the mat may vary depending on the moisture content of the fibrous materials or additives to the furnish. The effect of mat current is to hold the fibrous material to the . web and maintain desired alignment of fibres. Selective control of instantaneous polarity of the undersurface electrical conductor bars is provided along with selective placement in relation to the separate electric field-producing rods above the web.

Also, as shown in Fig. 2, a chamber 52 may be positioned below the web 12. As defined by wall structure 54, chamber 52 can extend over the full area of deposition. A fan 56 of any suitable design can be connected to chamber 52 to help prevent random escape of dust. A representative negative pressure level would be about 62.3 Pa (0.25 inch of water vacuum). This slight negative pressure may be used to conveniently reduce ambient dust about the structure without causing air turbulence forces in the flow-through chamber 24 which would adversely affect desired orientation of fibres. Orientation ratios can be reduced below desired levels at greater negative pressures.

Fig. 3 is an enlarged view of a portion of Fig. 2 showing the electrical field generated by charged rods 36 to 39 in predeterminedly spaced relationship above web 12. By use of opposite polarities in next adjacent rods 36 to 39, the field strength between the rods is increased to the algebraic sum of the voltages established in each rod. The on-site voltage available for these rods has an effect in selecting longitudinal spacing, i.e. along the mat-forming direction. Higher voltages permit greater longitudinal spacing between the rods.

The electric field includes lines of force extending substantially horizontally between the rods. For example, in a plane through the mid-points of rods 36 and 37, electric field lines of force extend parallel to the mat forming surface in the forming direction. Above and below these centre-plane lines of force, between the adjacent electrically conductive rods, electric field lines of force arch slightly, as indicated while maintaining alignment with the forming direction with a major component of the lines of force in parallel relation to the mat-forming surface.

The effect, generated by rotating the rods of the electric field on discrete fibres moving in the direction of mat 12 is represented in Fig. 4 which is an enlarged view of a portion of Fig. 2. Mat-forming surface 60 is presented by the mat 62 being formed on web 12; next adjacent rods 36 and 37 are of opposite polarity with rod 36 being positive and rod 37 being negative.

Fibres descend from upper portions of the flow-through chamber 24 along a flow path which is substantially normal to the web 12. In area 64, approaching the effective electric field, the fibres are. randomly oriented with axes of individual fibres in any of three dimensions; that is, individual fibres may be descending with their longitudinal axes at any angle between substantially normal to the plane of the web or substantially parallel to the plane of the web and also with their longitudinal axes at any angle between alignment with the direction of movement of the mat and 90° to that direction.

Fibres which are attracted to and adhere to the electrically charged rods are radially disposed in spoke-like fashion about each rod. This disposition of fibres adhering to the rods can be extended in length. Such fibre "whiskers" include fibres adhering to and extending longitudinally from a first tier of fibres in contact with the rods. As the rods rotate, in the direction shown, through the upper quadrants and through the quadrant approaching the mat-forming surface, these spoke-like protrusions of fibres become extended in length and closely adjacent. As the rotating rods take these adhering fibres through the final quadrant approaching the web 12, the fibres contact the mat-forming surface 60. Both the rotational centrifugal force and the continued rotation of the rods which causes fibre contact with the mat-forming surface 60 contribute to the breaking of the electrical attraction of the spoke-like fibres to the rods; these fibres are deposited with preferred direction orientation in the plane of the mat.

The direction of rod rotation is such that a rod and its adhering fibres, appear to "climb" the mat as it moves in the direction shown. The rods are positioned so that the bottom peripheral surface of each rod is contiguous to the surface of the mat being formed; because of attraction to the energized rods, the web 12 may be lifted slightly as it travels under a rod. The contiguous relationship clears fibres from the rods so that a portion of the first quadrant of a rod, after passage of its closest point to the mat surface, is initially free of fibres. The speed of rotation of the rods is selected to maximize orientation and avoid any build-up of fibres on the rods.

In addition to those fibres adhering to the rods, fibres falling towards and between the rods are subjected to the electric field generated by the rods, tending to orient fibres with their axes substantially parallel to the plane of the mat being formed and with their longitudinal axes in substantially the same direction as the direction of movement of web 12; such orientation is represented by the fibres in portion 66 of the chamber structure 24.

The subsurface electrical means, bars 44 to 49 as shown in Fig. 2, help maintain a separate electric force in the mat being formed by establishing a slight current in the mat.

Means for positioning, rotating, and electrically connecting the elongated electrically conductive rods are shown in Fig. 5. In this embodiment, a support frame 70 extends in the machine forming direction along opposite sides of the forming chamber 24. Support frame 70 holds the mounting and electrical contact bearings, e.g. 74, 75 at the leading ends and 76, 77 at the trailing end, for the axles 78, 79 and 80, 81, respectively, of the rods. As shown, the spacing between the web 12 and the rod axes increases in the direction of movement of web 12. Drive means 84 provides for controlled rotation of the rods.

Additional features which can be utilized to enhance fibre orientation at increased production rates while maintaining consistent results include: maximizing the electrostatic field strength while avoiding arcing, providing for maximizing the effect of the field strength including monitoring moisture content of the fibres and addition of materials to affect physical properties of the fibres, such as electrical conductivity, selection of the quantity, type, and state of binder resin included in the furnish, control of speed of rotation and size of the electrically conductive rods for producing the electric field, and control of the longitudinal movement of the conveyor support belt for the mat being formed.

The invention finds special application in working with lightweight fibrous materials. The pressure-refined wood furnish on which data is presented below had presented special problems to the prior art in obtaining desired orientation and commercial production rates. The wood is broken down closer to individual fibres in a pressurized steam refiner than under atmospheric attrition mill conditions. Various refining processes for preparing lightweight fibrous furnishes are known in the art (see e.g. "Modern Particleboard and Dry Process Fibreboard" by Thomas M. Maloney, pp. 98, 99, 212).

A predominant part of the bulk of pressurized steam refined wood furnish comprises extremely fine, hair-like fibres which can be less than 0.0254 mm (one mil) in diameter. These hair-like fibres can vary in length up to a much as 19 mm (three- fourths inch) but are predominantly about 6.35 to about 12.7 mm (one-quarter to one-half inch) in length. A tendency to cluster exhibited by the furnish, similar to that observed with cotton fibres, results from the nature of these extremely fine hair-like fibres. A significant percentage by weight of such pressurized disc refined furnish comprises heavier, elongated splinter-like pieces of wood having diameters up to about 0.0508 mm (two mils). Some of these exhibit fibre-like qualities being longitudinally pliable while others are more rigid. The balance of the weight of such furnish comprises dust-like particles.

Field strengths established by the rotating rods exhibiting voltage gradients of 101 to 404 volts per millimetre (2,500 to 10,000 volts/inch) provide suitable orientation conditions (the voltage gradient in volts per millimetre is equal to the positive polarity voltage at any instant supplied to an electrode plus the negative polarity voltage supplied at that instant to an adjacent electrode divided by the distance in millimetres between the electrodes). The voltage supply can be conventional; while AC or DC can be operational, DC is preferred because of better fibre orientation results. The voltage gradient should stay below the point where arcing can take place. The voltage gradient where arcing can take place in air varies from about 473 to about 670 volts per millimetre (12,000 to 17,000 volts/inch) depending on the relative humidity. Also current leakage increases more rapidly at field strengths above 404 volts per mm. A typical voltage gradient when working with lightweight furnish is about 315 volts per millimetre (8,000 volts/inch).

Control of rod spacing along the machine forming direction of the electrically charged rods above the web is partially dependent on the high voltage power supply connections. The field strength can be increased by utilizing two voltage power supplies of opposite polarity connected to adjacent rods. With 50,000 volt D.C. power supplies and 216 mm (eight and one-half inches) spacing between the rods in the machine forming direction, a voltage gradient up to about 473 volts per millimetre can be achieved. The voltage output of the power supply is adjustable. With lower voltage output capability, the spacing between the rods can be reduced to maintain the desired voltage gradients. Orientation ratio increases gradually in a substantially linear fashion as the voltage gradient increases.

Within the above range of values, rod diameter of about 19 mm (three quarters of an inch) provides optimum orientation results. Smaller or larger diameter rods, e.g. from about 12.7 mm, can be used. However, use of rods of 31.8 mm (one and one-quarter inches) diameter and larger, can result in lower orientation ratios with the lightweight wood furnish described. The nature of the rod metallurgy has little effect as long as the rod is a good conductor. Rod rotation, with the lightweight furnish described, is controlled in the range of about 100 to 300 r.p.m.

The improved orientation ratios and production rates are made available over a significantly wider range of moisture contents of the lightweight pressure refined furnish than what was previously considered practical with planar electrodes of the wall and partition type. For example, improved orientation ratios are available with moisture contents from about 5% to about 15% by weight. This significantly increases permissive selectivity available in the furnish and in the resin binder system used while maintaining consistency of results. With the chamber wall and partition type of electrodes of the prior art, the range of moisture contents of the furnish which could be used was more restricted; little orientation effect could be produced when the moisture content varied below an optimum percentage; e.g. 15% or higher moisture contents were generally considered to be better suited for obtaining orientation.

In practice of the present invention, moisture contents in the range of about 7-1/2% to about 10% are preferred although desired orientation ratios can be achieved over a much wider range of moisture contents. It has been found, however, that as moisture content approaches 20%, adhesiveness or so-called "tack-level" of certain resins can interfere with proper mat formation. Moisture content of the furnish, using conventional measuring means, can be monitored for better selection of electric field strength. Moisture content monitoring means can be mounted along the furnish handling line to activate a water spray solenoid valve to hold moisture content during periods when very low moisture content is exhibited by the particular furnish.

In practice, a variety of suitable binder systems exists which do not significantly inhibit achievement of proper orientation. Resin types include urea formaldehyde, phenol formaldehyde, isocyanate, and tannin formaldehyde. The resins can be applied in powder or liquid form. Percent of resin may typically run from about 4% to about 10% by weight of the dry fibre depending on the application and the product. Some liquid resins, such as urea formaldehyde, may cause tack and consequent clumping or balling of the fibres. Lower tack resins can be selected to avoid problems which could interfere with proper alignment and uniform deposition.

The effect of the electric field on the furnish can be modified, e.g. by controllably adding a salt, which enhances conductivity, to the fibrous material in order to improve orientation ratios. When the manufacturing process requires very low moisture contents, inclusion of a salt, such as sodium chloride, is beneficial. However, for most applications the moisture content preferred in the particular fibreboard manufacturing process provides adequate conductivity for desired orientation when using the method of the present invention.

While numerous factors can enter into evaluating characteristics of directionality in fibreboard, bending stiffness, also referred to as the modulus of elasticity in bending, provides a convenient measure of effective fibre orientation ratio achievement. Methods and means for measurement of the properties of oriented particleboard are known in the art; see e.g. "Electrically Aligned Particleboard and Fibreboard" by John W. Tal- bott, presented at the Eighth Washington State University Symposium of Particleboard of March 1974.

With random orientation, the ratio of particles in the "X" direction (direction of forming) to the number of particles in the "Y" direction (perpendicularly transverse to the direction of forming) is one to one. With fibre orientation in the direction of forming, this ratio increases. The index of the degree of orientation achieved with fibres is _ based on the ratio of the modulus of elasticity in the cross machine forming direction (Eₓ) to the modulus of elasticity in the cross machine direction (Ey). Ratios (EₓₗEy) of 1.2:1 and higher are achieved through use of the method of the present invention with pressure-refined wood furnish which has been considered the most difficult to handle of the lightweight furnishes described.

It has been demonstrated that the present invention is capable of providing desired orientation ratios with the lightweight furnish, produced by pressurized refining, at economically acceptable production rates over commercially practical forming areas. For example at an 8170 kg per hour (18,000 Ibs per hour) flow rate of furnish, electric field fibre orientation to desired ratios can readily be achieved when depositing fibres from 0.081 to about 0.407 kg m-² s⁻¹ (one to above five Ibs per square foot per minute) over a deposition surface of about 6.96 m² (seventy-five square feet).

With a flow rate of about 27.6 kg _{S}-¹ (300 Ibs per minute) and a deposition area of about 6.96 m², fibreboard having 801 kg m-³ (fifty Ib per cubic foot) density and a 3.18 mm (one-eighth inch) thickness after curing can be formed with desired orientation ratios at the rate of 0.254 m _{S}-¹ (fifty linear feet per minute). When the final thickness desired is 6.35 mm (one-fourth inch), such fibreboard can be produced at 0.127 m _{S}-¹ (twenty-five linear feet per minute). In practice, the actual deposition rate of the dry fibre exceeds such figures since pre-cured deposition of furnish will ordinarily be in excess of press capacity. For purposes of more efficient handling and more uniform distribution of fibres, the furnish is provided, distributed, oriented, and deposited at an optimum rate and, where the deposition exceeds press capacity, a portion of the mat can be shaved off prior to entry into the curing press and returned to the furnish supply and distribution line.

While specific structure, physical characteristics, and dimensional values have been set forth for purposes of describing one particular embodiment, it should be recognized that, in the light of the above description, modifications within the scope of the invention as claimed will be available to those skilled in the art.

## Claims

1. Continuous-line method for orienting and depositing lightweight furnish, including fibrous material with curable binder, in the manufacture of fibreboard having directional properties, in which a web presenting an extended surface area for deposition of furnish is moved continuously in a forming direction, and lightweight furnish, including elongated fibres moving along a flow path which is substantially normal to said surface for deposition of furnish, is guided towards said web, and in which said fibres being so guided and deposited are oriented by utilizing electrical forces, tending to orient longitudinal axes of the elongated fibres in parallel relationship to the plane of the mat being formed and aligned with the forming direction, and said electrical forces are produced by virtue of electrical potentials established between a plurality of elongate roller electrodes disposed transversely to the forming direction and in spaced relationship from each other along the forming direction, the roller electrodes being disposed adjacent to the mat being formed, characterised in that the roller electrodes are controllably rotated about their respective axes at a speed coordinated with the rate of longitudinal movement of the web to deposit onto the mat being formed fibres which have been attracted to the roller electrodes and have adhered to the roller electrodes.

2. A method as claimed in claim 1, in which the electrically charged rotating roller electrodes are predeterminedly positioned above the moving web in the direction of approach of fibres, with spacing above the moving web of roller electrodes located towards the leading longitudinal end of the area of fibre deposition being greater than corresponding spacing of the roller electrodes located towards the trailing longitudinal end of the area of fibre deposition to maintain a substantially uniform spacing between respective roller electrodes and adjacent mat-forming surface being presented by the web in travelling from the trailing longitudinal end towards the leading longitudinal end of the area of deposition.

3. A method as claimed in claim 1 or 2, in which electrical potential and polarity in said roller electrodes are controlled in order to control electric field strength longitudinally of the web.

4. A method as claimed in any of claims 1 to 3, in which elongated electrically conductive bars, positioned beneath the web with their longitudinal axes in transverse relationship to the longitudinal axis of the web and distributed longitudinally along the web in contact with the surface of the web opposite to the surface of deposition of furnish, are controllably energized to establish a current in the mat being formed.

5. Apparatus for carrying out the method of claim 1 in the continuous-line manufacture of fibreboard from lightweight furnish including fine textured elongated fibres and curable binding material, comprising a forming conveyor including a continuously moving web (12) presenting an extended surface area for deposition of furnish, means (14, 16, 18, 20, 22, 24) for establishing a flow path and delivering the furnish for deposition with the fibres in discrete form substantially free of fibre clusters, a plurality of elongated electrically conductive roller electrodes (36 to 41) located in the flow path of the furnish towards the surface area for deposition and in pre-selected spaced relationship above the surface area for deposition, the roller electrodes (36 to 41) being mounted with their longitudinal axes in transverse relationship to the direction of movement of the surface area for deposition and in substantially parallel relationship to such surface area, whereby the roller electrodes are adjacent to a mat-forming surface presented by deposition of fibres on the surface area for deposition, and being spaced along the direction of movement of such surface area across the flow path of furnish in approaching deposition, and means for applying an electrical potential to the roller electrodes for establishing an electric field having lines of force which tend to align longitudinal axes of the fibres with the direction of movement of the surface of deposition and into substantially parallel relationship with the mat-forming surface, characterised in that the apparatus includes means for controlling the electrical potential of the roller electrodes (36 to 41) and means (84) for rotating the roller electrodes (36 to 41) at a speed coordinated with the speed of movement of the web (12) such that elongated fibres adhering electrostatically to the roller electrodes contact the .mat-forming surface upon rotation of the roller electrodes.

6. Apparatus as claimed in claim 5, further including a plurality of elongated electrically conductive bars (44 to 49) located in under surface contact with the continuously moving web (12), the longitudinal axes of the elongated electrically conductive bars being in transverse relationship to the direction of movement of such web and in parallel relationship to the surface area for deposition, and means for establishing electrical potential in said bars (44 to 49) to establish an electric current in the mat being formed on the surface area for deposition.

7. Apparatus as claimed in claim 5 or 6, in which the means for establishing a flow path provide substantially uniform lateral and longitudinal distribution controlled flow of furnish as substantially individualized fibres moving towards the web for orientation and deposition purposes, and include guide wall means defining a flow-through structure (24) for passage of furnish towards the web, the flow-through structure (24) having cross-sectional lateral and longitudinal dimensions measured transversely to the flow path of furnish, which dimensions are correlated with corresponding dimensions of the deposition area for the fibres, the roller electrodes (36 to 41) being located in said flow-through structure.

8. Apparatus as claimed in claim 7, in which the guide wall means define leading and trailing longitudinal ends (32, 34) of the mat forming surface presented for deposition of fibres with the roller electrodes (36 to 41) being located towards the leading longitudinal end (32) being spaced a greater distance from the web (12) than roller electrodes located towards the trailing longitudinal end (34).

## Patentansprüche

1. Kontinuierliches Verfahren zum Ausrichten und Ablagern einer leichtgewichtigen Eintragsmasse, in der sich faseriges Material mit härtbarem Binder befindet, zum Herstellen einer Faserplatte mit Richtcharakteristik, bei dem eine eine ausgedehnte Oberfläche zum Ablagern der Eintragsmasse bietende Bahn kontinuierlich in eine Formrichtung bewegt wird und leichtgewichtige Eintragsmasse, die einschließlich länglicher Fasern entlang einem Strömungsweg bewegt wird, die im wesentlichen normal zu der genannten Fläche zum Ablagern der Eintragsmasse ausgerichtet ist, in Richtung auf die Bahn geführt wird, und bei dem die so geführten und abgelagerten Fasern unter Verwendung von elektrischen Kräften ausgerichtet werden, indem die Längsachsen der länglichen Fasern in parallelem Verhältnis zu Ebene der Matte ausgerichtet werden, die in der Formrichtung ausgerichtet und ausgebildet wird, wobei die elektrischen Kräfte aufgrund elektrischer Potentiale erzeugt werden, die zwischen einerVielzahl von länglichen Rollenelektroden eingerichtet werden, die quer zur Formrichtung und in dieser Formrichtung im beabstandeten Verhältnis zueinander angeordnet sind, welche Rollenleketroden neben der auszubildenden Matte angeordnet sind, dadurch gekennzeichnet, daß die Rollenelektroden steuerbar um ihre jeweiligen Achsen mit einer Geschwindigkeit gedreht werden, die mit dem Ausmaß der Längsbewegung der Bahn koordiniert ist, um auf die auszubildende Matte Fasern abzulagern, die von den Rollenelektroden angezogen worden sind und an den Rollenelektroden haften.

2. Verfahren nach Anspruch 1, bei dem die elektrisch-geladenen, sich drehenden Rollenelektroden vorbestimmt oberhalb der sich bewegenden Bahn in Annäherungsrichtung der Fassern positioniert sind, und zwar mit einem Abstand oberhalb der sich bewegenden Bahn, welcher Abstand hinsichtlich der Rollenelektroden, die in Richtung auf das führende Längsende des Bereiches der Faserablagerung angeordnet sind, größer ist als der entsprechende Abstand der Rollenelektroden, die in Richtung auf das hintere längliche Ende des Bereiches der Faserablagerung angeordnet sind, um in Bewegungsrichtung vom hinteren länglichen Ende in Richtung auf das führende längliche Ende des Ablagerungsbereiches einen im wesentlichen gleichförmigen Abstand zwischen den jeweiligen Rollenelektroden und der von der Bahn dargebotenen benachbarten Mattenformfläche aufrechtzuerhalten.

3. Verfahren nach Anspruch 1 oder 2, bei dem das elektrische Potential und die Polarität in den genannten Rollenelektroden gesteuert werden, um die elektrische Feldstärke entlang der Bahn zu steuern.

4. Verfahren nach einem der Ansprüche 1 bis 3, bei dem längliche, elektrisch-leitende Stangen, die unterhalb der Bahn so angeordnet sind, daß ihre Längsachsen im Querverhältnis zur Längsachse der Bahn verlaufen, und die in Längsrichtung entlang der Bahn in Berührung mit der Fläche der Bahn verteilt sind, die der Ablagerungsfläche der Eintragsmasse entgegengesetzt ist, steuerbar unter Strom gesetzt werden, um in der auszubildenden Masse einen Stromfluß zu erzeugen.

5. Apparat zum Durchführen des Verfahrens nach Anspruch 1 zum kontinuierlichen Herstellen einer Faserplatte aus leichtgewichtiger Eintragsmasse einschließlich feiner, texturierter, länglicher Fasern und einem härtbaren Bindematerial, mit einem Formförderer einschließlich einer kontinuierlich sich bewegenden Bahn (12), die einen ausgedehnten Flächenbereich zum Ablagern einer Eintragsmasse bietet, mit Mitteln (14,16,18, 20, 22, 24) zum Einrichtung eines Strömungsweges und zum Abgeben der Eintragsmasse zum Ablagern derselben mit den Fasern in diskreter Form, die im wesentlichen frei von Faserklumpen ist, mit einer Vielzahl von länglichen, elektrisch-leitenden Rollenelektroden (36-41), die auf dem Strömungsweg der Eintragsmasse in Richtung auf den Oberflächenbereich für die Ablagerung und im vorausgewählten Abstandsverhältnis oberhalb der Ablagerungsfläche liegen, welche Rollenelektroden (36-41) mit ihren Längsachsen im Querverhältnis zur Bewegungsrichtung der Ablagerungsfläche und in wesentlichen im parallelen Verhältnis zu solch einem Oberflächenbereich angebracht sind, wodurch die Rollenelektroden neben einer Mattenformfläche liegen, die durch das Ablagern der Fasern auf die Ablagerungsfläche gebildet ist und wodurch die Rollenelektroden entlang der Bewegungsrichtung dieses Flächenbereiches quer über den Strömungsweg der Eintragsmasse mit näherkommender Ablagerung beabstandet sind, und mit Mitteln zum Anlegen eines elektrischen Potentials an die Rollenelektroden zum Einrichten eines elektrischen Feldes mit Kraftlinien, die dazu neigen, die Längsachsen der Fasern mit der Bewegungsrichtung der Ablagerungsfläche und im wesentlichen im parallelen Verhältnis mit der Mattenformfläche auszurichten, dadurch gekennzeichnet, daß der Apparat Mittel zum Steuern des elektrischen Potentials der Rollenelektroden (36―41) und Mittel (84) zum Drehen der Rollenelektroden (36―41) mit einer Geschwindigkeit umfaßt, die mit der Bewegungsgewindigkeit der Bahn (12) so koordiniert ist, daß die elektrostatisch an den Rollenelektroden haftenden länglichen Fasern die Mattenformfläche bei der Drehung der Rollenelektroden berühren.

6. Apparat nach Anspruch 5, welcher weiterhin eine Vielzahl von länglichen elektrisch-leitenden Stangen (44 bis 49) umfaßt, welche unterhalb der kontinuierlich sich bewegenden Bahn (12), diese berührend angeordnet sind, wobei die Längsachsen der länglichen, elektrisch leitenden Stangen im Querverhältnis zur Bewegungsrichtung einer solchen Bahn und in parallelem Verhältnis zur Ablagerungsfläche liegen, und daß der Apparat weiterhin Mittel zum Einrichten eines elektrischen Potentials in diesen Stangen (44-49) umfaßt, um in der auf der Ablagerungsfläche auszubildenden Matte einen elektrischen Strom einzurichten.

7. Apparat nach Anspruch 5 oder 6, bei dem die Mittel zum Einrichten eines Strömungsweges einen im wesentlichen gleichförmigen, seitlich und in Längsrichtung verteilten, gesteuerten Eintragsmassenstrom als im wesentlichen individualisierte Fasern vorsehen, die sich zum Ausrichten und Ablagern in Richtung auf die Bahn bewegen, und daß der Apparat FÜhrungswandmittel umfaßt, die ein Durchflußgebilde (24) für die Passage in der Eintragsmasse in Richtung auf die Bahn bilden, welches Durchflußgebilde (24) quer zum Strömungsweg der Eintragsmasse gemessene seitliche und Längsquerschnittsdimensionen hat, welche mit entsprechenden Dimensionen des Ablagerungsbereiches für die Fasern in Beziehung stehen, wobei die Rollenelektroden (36―41) in diesem Durchflußgebilde angeordnet sind.

8. Apparat nach Anspruch 7, bei dem die Führungswandmittel führende und hintere Längsenden (32, 34) der Mattenformfläche bilden, die sich für das Ablagern der Fasern darbieten, wobei die Rollenelektroden (36-41) in Richtung auf das führende Längsende (32) in einem größeren Abstand zur Bahn (12) angeordnet sind, als die Rollenelektroden, welche in Richtung auf das hintere Längsende (34) angeordnet sind.

## Revendications

1. Procédé continu pour orienter et déposer une matière légère, comprenant une matière fibreuse et un liant durcissable, dans la fabrication de panneaux de fibres à caractéristiques directionnelles, dans lequel une feuille présentant une surface étendue de dépôt de matière est déplacée de façon continue dans une direction de formage, et une matière légère, comprenant des fibres allongées en déplacement le long d'un passage d'écoulement qui est sensiblement perpendiculaire à ladite surface de dépôt de matière, est guidée vers la feuille, et dans lequel les fibres ainsi guidées et déposées sont orientées par utilisation de forces électriques tendant à orienter les axes longitudinaux des fibres allongées parallèlement au plan de la natte en formation et en alignement avec la direction de formage, ces forces électriques étant engendrées au moyen de potentiels électriques établis entre une pluralité d'électrodes à rouleau allongées disposées transversalement à la direction de formage et à distance les unes des autres dans la direction de formage, les électrodes à rouleau étant placées près de la natte en formation, caractérisé en ce que les électrodes à rouleau sont commandées en rotation autour de leurs axes respectifs à une vitesse liée à la vitesse de déplacement longitudinal de la feuille, de manière à déposer sur la natte en formation les fibres qui ont été attirées sur les électrodes à rouleau et ont adhéré aux électrodes à rouleau.

2. Procédé suivant la revendication 1, dans lequel les électrodes rotatives à rouleau, électriquement chargées, sont placées à des positions prédéterminées au-dessus de la feuille mobile, dans la direction d'approche des fibres, la dis-. tance au-dessus de la feuille mobile pour les électrodes à rouleau situées vers l'extrémité longitudinale avant de la zone de dépôt de fibres étant plus grande que la distance correspondante des électrodes à rouleau situées vers l'extrémité longitudinale arrière de la zone de dépôt de fibres, de manière à maintenir un espacement sensiblement constant entre les électrodes à rouleau respectives et la surface adjacente de formation de natte présentée par la feuille en déplacement de l'extrémité longitudinale arrière vers l'extrémité longitudinale avant de la zone de dépôt.

3. Procédé suivant la revendication 1 ou 2, dans lequel le potentiel électrique et la polarité des électrodes à rouleau sont déterminés de manière à régler l'intensitérique dans la direction longitudinale de la feuille.

4. Procédé suivant l'une quelconque des revendications 1 à 3, dans lequel des barreaux allongés, électriquement conducteurs, placés sous la feuille avec leurs axes longitudinaux disposés transversalement à l'axe longitudinal de la feuille, et répartis longitudinalement le long de la feuille en contact avec la surface de la feuille qui est à l'opposé de la surface de dépôt de matière, sont mis sous tension de façon réglable, pour établir un courant dans la natte en formation.

5. Appareil pour la mise en oeuvre du procédé de la revendication 1, dans la fabrication en continu de panneaux de fibres au moyen d'un matériau léger comprenant des fibres allongées à texture fine et une matière de liaison durcissable, qui comprend un transporteur de formage comportant une feuille (12) en mouvement continu qui présente une surface étendue de dépôt de matériau, des moyens (14, 16, 18, 20, 22, 24) qui définissent un conduit d'écoulement et distribuent le matériau pour le déposer avec les fibres à l'état séparé et sensiblement sans amas de fibres une pluralité d'électrodes à rouleau (36 à 41), allongées, électriquement conductrices, placées dans le passage du matériau vers la surface de dépôt et à distance prédéterminée au-dessus de la surface de dépôt, les électrodes à rouleau (36 à 41) étant montées avec leurs axes longitudinaux disposés transversalement à la direction de mouvement de la surface de dépôt et sensiblement parallèlement à cette surface, de sorte que les électrodea à rouleau sont adjacentes à une surface de formation de natte, engrendrée par le dépôt des fibres sur la surface de dépôt, et sont espacées le long de la direction de déplacement de cette surface à travers le passage de matériau qui va se déposer, et des moyens d'application d'un potentiel électrique aux électrodes à rouleau pour créer un champ électrique dont les lignes de force tendent à aligner les axes longitudinaux des fibres avec la direction de déplacement de la surface de dépôt et sensiblement parallèlement à la surface de formation de natte, caractérisé en ce que l'appareil comprend des moyens de commande du potentiel électrique des électrodes à rouleau (36 à 41) et des moyens (84) de mise en rotation des électrodes à rouleau (36 à 41) à une vitesse liée à la vitesse de déplacement de la feuille (12), de manière à ce que les fibres allongées qui adhèrent électrostatiquement aux électrodes à rouleau viennent en contact avec la surface de formation de natte lors de la rotation des électrodes à rouleau.

6. Appareil suivant la revendication 5, qui comprend une pluralité de barreaux allongés (44 à 49), électriquement conducteurs, placés en contact avec la surface inférieure de la feuille (12) en mouvement continu, les axes longitudinaux des barreaux allongés électriquement conducteurs étant disposés transversalement par rapport à la direction de déplacement de cette feuille et parallèlement à la surface de dépôt, et des moyens d'établissement d'un potentiel électrique dans les barreaux (44 à 49) de manière à établir un courant électrique dans la natte en formation sur la surface de dépôt.

7. Appareil suivant la revendication 5 ou 6, dans lequel les moyens qui définissent un passage d'écoulement assurent un débit réglé de matériau, à répartition latérale et longitudinale sensiblement uniforme, sous la forme de fibres sensiblement individualisées se déplaçant vers la feuille pour des raisons d'orientation et de dépôt, et comprennent des parois de guidage définissant une structure de traversée (24) pour la passage du matériau vers la feuille, la structure de traversée (24) ayant en section transversale des dimensions latérales et longitudinales mesurées transversalement au passage d'écoulement du matériau, ces dimensions étant en corrélation avec le dimensions correspondantes de la surface de dépôt des fibres, les électrodes à rouleau (36 à 41) étant situées dans ladite structure de traversée.

8. Appareil suivant la revendication 7, dans lequel les parois de guidage définissent les extrémités longitudinales avant et arrière (32, 34) de la surface de formation de natte présentée pour le dépôt des fibres, les électrodes à rouleau (36 à 41) situées vers l'extrémité longitudinale avant (32) étant plus éloignées de la feliille (12) que les électrodes à rouleau situées vers l'extrémité longitudinale arrière (34).
